

# UNITED STATES PATENT OFFICE.

CHRISTOPHER J. HEIDORF, OF HUDSON FALLS, NEW YORK.

## WALL-PAPER FINISH.

1,353,473.

Specification of Letters Patent. Patented Sept. 21, 1920.

No Drawing. .

Application filed October 23, 1918. Serial No. 259,411.

*To all whom it may concern:*

Be it known that I, CHRISTOPHER J. HEIDORF, a citizen of the United States, residing at Hudson Falls, in the county of Washington, State of New York, have invented certain new and useful Improvements in Wall-Paper Finish; and I do hereby declare the following to be a full, clear, and exact description of the invention, such as will enable others skilled in the art to which it appertains to make and use the same.

This invention relates to new and useful improvements in wall papers and particularly to coatings therefor.

One object of the present invention is to provide a novel and improved coating for a wall paper which will render the surface of the paper ornamental and attractive.

Another object is to provide a novel coating for a wall paper whereby the paper is rendered readily capable of being washed.

A still further object of the present invention is to provide a novel and improved coating which can be applied to any common wall paper to render the same fire-proof and washable.

Other objects and advantages will be apparent from the following description.

The paper is of any suitable kind, such as is ordinarily used to cover walls and ceilings of houses. The coating consists of a mixture of ground mica, shellac, and casein, or casein glue, to which the proper proportion of water is mixed to produce the de-

sired consistency for spreading on the paper with a brush. This coating may be applied by any of the well known coating machinery, now used, before the paper is placed on the market, or the coating may be applied to the paper after it has been pasted to the wall and ceiling.

The glue and the shellac render a fine gloss to the surface of the paper, and at the same time water-proofs the paper. This also renders the paper capable of being easily cleansed by the application of a sponge or wet rag or cloth, with the addition of such cleansing materials as soap, or cleaning powders, without damage to the paper.

The ground mica is applied to the paper first, and then the desired design printed thereon, on top of the mica, after which the paper is passed through a ground machine and a second coating of ground mica applied, together with a solution consisting of casein or casein glue, and shellac to produce the required gloss to the paper.

What is claimed is:

A coating composition comprising casein, shellac, and ground mica.

In testimony whereof, I affix my signature, in the presence of two witnesses.

CHRISTOPHER J. HEIDORF.

Witnesses:

KATHRYN M. FLANIGAN,  
WILLIAM I. LOCKE.